

## UNITED STATES PATENT OFFICE

SHINJIRO HORII, OF KANDA-KU, TOKYO, JAPAN

## STENCIL SHEET

No Drawing. Application filed August 1, 1930, Serial No. 472,500, and in Japan June 28, 1930.

My invention relates to improvements in stencil sheets for use in duplicating manuscript and typewritten documents, drawings and the like consisting of a fibrous base having a coating which is impermeable to ink, and adapted to be stencilized by the pressure of a hand stylus or by the impact of the type of a typewriting machine.

It has previously been proposed to produce a stencil sheet of a fibrous base, such as Japanese yoshino paper, coated or impregnated with a coating material including esters of polysaccharides and a tempering agent, such as naphthenic acid glycerides, chlorinated naphthalene, fatty acid of Tsubaki oil or a mixture of them.

It has also been proposed to produce a stencil sheet of loose-fibered tissue coated with cellulose acetate plastified and stabilized by acetanilid, combined with a softening agent, such as glycerine and diethyl phthalate.

According to the present invention the stencil sheet comprises a base of fibrous material having a coating including esters of polysaccharides, a metallic soap of naphthenic acid, a suitable tempering agent.

A metallic soap of naphthenic acid is prepared by heating and combining together the equivalent portions of naphthenic acid and an oxide of metal, or by the double-decomposition of a solution of an alkali soap of naphthenic acid with a solution of some salt of metals, such as aluminum, iron, calcium or magnesium.

The film of cellulose esters as well as of the other esters of polysaccharides, however, is highly unstable and considerable deteriorates when stored for a long period of time. Moreover, it is extremely sensitive to sunlight. A clear film exposed for a few days only becomes brittle so that it will not withstand mild bending even without cracking. The use of oils and plasticizers will extend the life, but eventually failure will occur. The fatty oils become rancid on exposure and make the film sticky. Consequently, a stencil sheet having such a coating is unstable for

use in many climates. The esters of polysaccharides generally contain some residual acid, and the solution of the esters may be acid either from this case or from the solvents employed. The acidity of the esters and the rancidity of the fatty oils or fatty materials decrease the colloidal property of the esters and increase the chemical decomposition of the esters.

It is common practice to neutralize the free acid and the acid which may be produced afterwards with feeble alkalies, such as urea and other amines, but these substances make them unsafe because of producing a harmful product which decreases the colloidal property of the esters, and acts to decompose the esters, as the majority of the stabilizing materials exert an alkaline reaction upon the esters. The choice of the stabilizing material is in practice preferably restricted to such as will not harmfully affect the coating of the stencil sheet of the kind above referred to. Now, it has been found that metallic soaps of naphthenic acid, for example calcium naphthenate, will overcome the above defects.

The metallic soaps of naphthenic acid are the most effective stabilizers for the esters of polysaccharides. They exert no adverse action on the esters of polysaccharides and combine with the free acid present in the esters, forming salts of the metals involved and liberating the naphthenic acid. The naphthenic acid produced is a feeble acid of saturated constitution and exerts no saponifying action on the esters of polysaccharides, improving the durability and toughness of the cellulosic film. Metallic soaps of naphthenic acid and naphthenic acid also are the plasticizers for the esters of polysaccharides. Furthermore, it has been found to be more effective to use them in combination with an alkyl ester of naphthenic acid, e. g. ethyl or butyl ester, as the plasticizers of the esters of polysaccharides.

A metallic soap of oleic acid, preferably the sodium or potassium soap, has been suggested as a softening and stabilizing material in a cellulose ester stencil sheet with other

tempering agents, but the alkali soaps are weak alkalies, and they act on the cellulose esters, decreasing their colloidal property.

5 The alkali soaps of oleic acid combine with the free acid present in the cellulose esters, and there will be produced the salts of the metals and free oleic acid. The oleic acid is a stronger acid than naphthenic acid and is an unsaturated one. Consequently, it ac-

10celerates the rancidity of the oils present and also exerts the saponification of the cellulose esters of the coating. Therefore, the use of alkali soaps, or other soaps of fatty acids, gives no good results.

15 As already described, the stencil sheet produced in accordance with the present invention is very durable, owing to its stability, and the stencil is also remarkably soft and pliable because of the combined use of an alkyl ester of naphthenic acid with a metallic soap of naphthenic acid giving a clear stencil by the pressure of a writing machine.

In carrying out the invention into practice, first the esters of polysaccharides, such as 25 starch acetate, mannan acetate, cellulose acetate, cellulose stearate and cellulose nitrate, are dissolved in a volatile solvent, such as ether, alcohol, acetone, ethyl acetate, butyl acetate, butyl alcohol, benzine, benzol or a mixture of them, and then the solution is mixed with a solution of a metallic soap of naphthenic acid dissolved in a suitable solvent, such as a mixture of acetone and cyclohexanon, in admixture of ethyl or butyl naphthenate and other suitable tempering agents such as fatty oils, fatty acid of Tsubaki oil, liquid waxes, naphthenic acid glycerides, chlorinated naphthalene, paraffin oil, butyl phthalate and cresyl phosphate, and, if desired, some coloring substances such as pigments or dyes. Then the mixed solution is coated on a base material such as Japanese yoshino paper.

40 45 The proportions of the ingredients may vary according to several circumstances. By the way of example particulars are given as follows:—

#### Example I

|                            | Parts by weight |
|----------------------------|-----------------|
| Cellulose nitrate          | 20              |
| Alcohol                    | 20              |
| 55 Ethyl acetate           | 30              |
| Butyl acetate              | 10              |
| Calcium naphthenate        | 1-5             |
| Ethyl naphthenate          | 5               |
| Cyclohexanon               | 5-20            |
| 60 Benzol                  | 20              |
| Butyl phthalate            | 2               |
| Naphthenic acid glycerides | 15              |
| Tsubaki oil                | 10              |
| Fatty acid of Tsubaki oil  | 5               |
| 65 Paraffin oil            | 5               |

#### Example II

|                            | Parts by weight |
|----------------------------|-----------------|
| Cellulose acetate          | 15              |
| Mannan acetate             | 5               |
| Acetone                    | 50              |
| Cyclohexanon               | 10              |
| Ethyl acetate              | 20              |
| Calcium naphthenate        | 1-5             |
| Ethyl naphthenate          | 10              |
| Naphthenic acid glycerides | 10              |
| Chlorinated naphthalene    | 5               |
| Fatty acid of Tsubaki oil  | 5               |

The above coating compositions may be 80 diluted with any suitable solvents to the desired consistency.

The term "esters of polysaccharides" is intended to include not only one of definite esters of polysaccharides, but also a mixture 85 of them.

What I claim is:—

1. A stencil sheet adapted for stencilizing by pressure, comprising a base of fibrous material having a coating including esters of 90 polysaccharides, a metallic soap of naphthenic acid, and a tempering agent.

2. A stencil sheet adapted for stencilizing by pressure, comprising a base of fibrous material having a coating including esters 95 of polysaccharides, a metallic soap of naphthenic acid, an alkyl ester of naphthenic acid, and a tempering agent.

3. A stencil sheet adapted for stencilizing by pressure, comprising a base of fibrous 100 material having a coating including esters of polysaccharides, a metallic soap of naphthenic acid, ethyl naphthenate, and a tempering agent.

4. A stencil sheet adapted for stencilizing by pressure, comprising a base of fibrous material having a coating including esters of 105 polysaccharides, calcium naphthenate and a tempering agent.

5. A stencil sheet adapted for stencilizing by pressure, comprising a base of fibrous material having a coating including esters of 110 polysaccharides, calcium naphthenate, an alkyl ester of naphthenic acid, and a tempering agent.

6. A stencil sheet adapted for stencilizing by pressure, comprising a base of fibrous material having a coating including esters of 115 polysaccharides, calcium naphthenate, ethyl naphthenate, and a tempering agent.

In testimony whereof I affix my signature.

SHINJIRO HORII.